

**UNITED STATES PATENT OFFICE**

**2,520,748**

# **POLYMERIC OXIDE LUBRICANT CONTAINING ORGANIC DISULFIDE**

William E. Vaughan and Denham Harman,  
Berkeley, Calif., assignors to Shell Development  
Company, San Francisco, Calif., a corporation  
of Delaware

**No Drawing. Application October 28, 1946,  
Serial No. 706,097**

**10 Claims. (Cl. 252—48.2)**

This invention relates to novel lubricating compositions. More particularly, it pertains to certain fractions of non-mineral oil base sulfur-containing compounds, which are especially suitable for low temperature or extreme pressure lubrication.

The use of mineral oil fractions for lubricating is suitable for many purposes, but it is well known that such lubricants possess certain inherent limitations, such as tendency to oxidize, thickening at low temperatures, etc. A large number of additives have been employed with mineral oils in order to improve these shortcomings. To a certain degree, the resulting compositions may be used successfully for most lubricating purposes.

Various synthetic lubricants have been proposed from time to time. These include polymers of cracked wax olefins, alkylated aromatics such as alkylated naphthalenes, and so on. Some of these are useful for special purposes, but, especially if the previously known synthetic lubricants were derived from olefinic sources, they usually possessed corrosion and oxidation characteristics limiting their utility to a substantial degree.

Another type of synthetic lubricant which has been investigated is the alkylene oxide polymer type, such as polymerized propylene oxide. Such polymers are useful under mild operating conditions.

Organic disulfides, such as dimethyl disulfide, are known, but the possible use of certain classes of them as lubricants has not previously been proposed. Furthermore methods for the formation of such disulfides have been described, but heretofore the adjustment of such methods for the preparation of disulfides having lubricating properties has not been suggested.

It is an object of the present invention to provide a novel method for the production of a non-hydrocarbon lubricant. It is another object of the present invention to provide a novel method for the preparation of a lubricant useful at low temperatures. It is still another object of this invention to provide a novel method for the preparation of a lubricant possessing inherent extreme pressure properties. It is a further object of the present invention to provide synthetic lubricants derived from mixtures of mercaptans. It is yet another object of the present invention to utilize petroleum by-products. Another object is the provision of extreme pressure additives for other lubricants. Other objects will become evident from the following disclosure.

Now, in accordance with this invention, it has been found that lubricants having inherent extreme pressure properties may comprise organic disulfides having the general configuration

$$\text{XO}-\text{R}-\text{S}-\text{S}-\text{R}-\text{O}\text{X}$$

wherein R is an organic radical, and each X is a substituent such as a hydrogen atom, hydrocarbon radical or acyl group, especially if the disulfide or a mixture thereof has a minimum boiling point above about 140° C. at 0.2 cm. mercury pressure. Still in accordance with this invention, it has been found that, not only may such disulfides be used without modification as extreme pressure lubricants, but that they may be employed as extreme pressure additives for other lubricants. Disulfides satisfactory for such uses may be prepared, according to the present invention, by forming the metallic salts of a mercaptan, or mixture of mercaptans, oxidizing the salt, and removing the more volatile fraction of the product, which essentially is a disulfide or mixture of disulfides.

25 The mercaptans from which the subject lubricants may be prepared are those having the general formula

$$X-O-R_1-SH$$

30 wherein **X** is a substituent such as a hydrogen atom, a hydrocarbon group or an acyl radical, and **R**<sub>1</sub> is a hydrocarbon radical, preferably an alkylene radical. These include for example mercaptoethyl alcohol, mercaptopropyl alcohol, mercaptobutyl alcohol, mercaptoamyl alcohol, mercaptohexyl alcohol, mercaptoheptyl alcohol, mercaptooctyl alcohol, mercaptononyl alcohol, mercaptoodecyl alcohol, mercaptododecyl alcohol, etc. 35 wherein the sulphydryl and hydroxyl groups are at opposite ends of the hydrocarbon chain.

40 Although such a configuration is preferred for the preparation of the present disulfide lubricants, alternative configurations include those in which the hydrocarbon is highly branched and/or  
45 in which the sulphydryl group or the hydroxyl group (or both) is not on a terminal carbon atom.

group (or both) is not on a terminal carbon atom. Mercaptoalkyl alcohols having the latter type of configuration include 1-hydroxy-3-mercaptopbutane, 2-hydroxy-4-mercaptopbutane, 2-hydroxy-5-mercaptopentane, 3-hydroxy-4-mercaptopentane, 1-hydroxy-4-mercaptophexane, 2-hydroxy-6-mercaptophexane, 3-hydroxy-7-mercaptodecane, 1-hydroxy-3-methyl-6-mercaptophexane, 1-hydroxy-4-isopropyl-8-mercaptophexane, and their 50 homologs and analogs.

The ethers of mercapto alcohols which form satisfactory disulfide lubricants have the general configuration



wherein  $\text{R}_2$  and  $\text{R}_3$  are hydrocarbon radicals, particularly alkyl radicals. Preferably, the mercapto group and the ether radical  $-\text{O}-\text{R}_3$  are attached to opposite terminal carbon atoms of a saturated hydrocarbon. These include such ethers as 1-mercaptop-4-methoxybutane, 1-mercaptop-5-ethoxypentane, 1-mercaptop-4-ethoxybutane, 1-mercaptop-6-methoxyhexane, 1-mercaptop-6-ethoxyhexane, 1-mercaptop-6-propoxyhexane, etc. Such ethers may have branched hydrocarbon radicals. For example, suitable ethers of this type are 1-mercaptop-2-ethyl-3-methoxypropane, 1-mercaptop-3-methyl-4-ethoxybutane, 1-mercaptop-3-isopropyl-7-butoxyheptane, etc.

Other ethers which may be used to form satisfactory disulfide lubricants include those in which the mercapto group and/or the alkoxy group are attached to carbon atoms other than terminal carbon atoms. These are illustrated by such ethers as 1-mercaptop-2-methoxypropane, 1-mercaptop-3-ethoxybutane, 1-mercaptop-4-propoxyhexane, 1-mercaptop-5-butoxydecane, 2-mercaptop-3-methoxypropane, 3-mercaptop-4-ethoxybutane, 4-mercaptop-5-propoxypentane, 2-mercaptop-3-methoxybutane, 3-mercaptop-5-ethoxyhexane, 2-mercaptop-3-ethyl-4-methoxypentane, etc.

Esters of mercapto alcohols likewise may be used for the formation of the disulfide lubricants described herein. These have the general formula



wherein  $\text{R}_4$  and  $\text{R}_5$  are hydrocarbon, especially alkyl, radicals. Preferred esters having the above configuration include those in which the mercapto group and the ester group are attached to terminal carbon atoms of a hydrocarbon. The esters from which the most satisfactory disulfide lubricants are prepared are those in which  $\text{R}_7$  is a saturated aliphatic hydrocarbon radical having less than 13 carbon atoms. These include such esters as 1-mercaptop-3-methoxyloxypropane, 1-mercaptop-4-ethoxyloxybutane, 1-mercaptop-5-butoxyloxypentane, 1-mercaptop-6-(2-ethylhexyloxy) hexane and their homologs and analogs.

The esters may have other configurations wherein the sulphydryl group, the ester group or an alkyl group is attached to carbon atoms which are not terminals of a hydrocarbon chain. Typical esters having such configurations are 1-mercaptop-2-methoxyloxypropane, 1-mercaptop-4-ethoxyloxyhexane, 2-mercaptop-3-propoxyloxypropane, 3-mercaptop-5-ethoxyloxypentane, 2-mercaptop-5-methoxyloxyhexane, 1-mercaptop-2-methyl-3-methoxypropane, etc.

As noted hereinbefore, the disulfide lubricants may be prepared by oxidizing a metallic salt of the mercaptan. The metal salt is conveniently formed by treatment of mercaptans such as those above with a normal metallic oxide or hydroxide, preferably in the presence of water. Suitable oxides, carbonates and hydroxides are, for example, those of the alkali metals and the alkaline earth metals, and include lithium, sodium, potassium, calcium, strontium and barium oxides, carbonates and hydroxides.

The metal salts are conveniently prepared by dissolving the metal compound in water and adding the mercaptan (or mercaptans) thereto. This may be done at room temperature, but other temperatures from about 10° C. to about 100° C. may be employed. The reaction is quantitative and usually proceeds substantially instantaneously, although some of the less active mercaptans may require a more prolonged period to allow complete transformation of the mercaptans to the metallic salt.

Following the completion of the above reaction, the salts so formed are oxidized to form the disulfide. This may be done conveniently in the same alkaline medium in which the salt was formed, an excess of alkali being present. Alternatively, the salt may be isolated and subsequently placed in another medium for treatment with oxidizing agents. Preferably any medium used is alkaline, and may be made so with inorganic alkalies, such as those described above. Alternatively the oxidation may be conducted in the presence of an organic base, such as primary, secondary or tertiary amines, pyridine, piperidine or quaternary ammonium bases or their salts. The medium may be aqueous or organic, such as alcoholic.

The oxidation of the metallic salt of the mercaptan is effected by use of oxidizing agents, such as air, oxygen, ozone, iodine, bromine, chlorine, hydrogen peroxide, organic peroxides, permanganate, dichromate, etc. The reaction usually is conducted by gradual addition of the oxidizing agent to a suspension or solution of the mercaptan salt. This is done conveniently starting at room temperature, although temperatures between about -40° C. to about 150° C. may be used, dependent upon the reactivity of the oxidizing agent and the mercaptan salt. The addition of the oxidizing agent may be conducted at a relatively rapid rate if temperature control methods are employed. Preferably, however, the addition is conducted over a more extended period, that is, from about one to about forty-eight hours. With such reactive mercaptan salts as the potassium salt of gamma-mercaptopropyl alcohol, the reaction is complete in two to eight hours, when iodine is the oxidant, the reaction temperature being about 20-30° C. An equivalent amount of the oxidizing agent, or an excess thereof, must be used in order to obtain complete oxidation of the salt to the disulfide.

An essential feature of the present invention is the substantially complete removal of volatile components from the product. This is especially important when mixtures of mercaptans, such as those derived from petroleum sources, are used for the preparation of the disulfide. Such mixtures may include inert volatile material or lower mercaptans which form disulfides having too high a volatility to be useful for most lubricating purposes. The source of mercaptans and their configurations will have a great effect upon the proportion of relatively volatile components in the product.

The fraction of relatively volatile constituents removed will depend upon the lubricating purpose for which the remainder will be employed. If no fraction is removed the composite product is generally useless as a lubricant, since the lighter fractions will inevitably volatilize during operation to a greater or less degree dependent upon the conditions to which it is subjected. However, for general lubricating purposes, the fraction volatilizing below about 140° C. at 0.2

cm. mercury pressure is preferably removed, and generally, that fraction volatilizing below about 120° C. at 0.2 cm. mercury pressure is removed in order to obtain a lubricant having optimum properties.

The product may be further treated to remove color or alter configuration. For example, instead of forming bis(alkoxyalkyl)disulfides or bis(alkoxyloxyalkyl)disulfides from the corresponding mercaptans, as described above, bis(hydroxyalkyl)disulfides may be prepared from the corresponding mercaptan, after which the disulfide may be etherified or esterified.

Various etherifying agents may be used for etherifying terminal hydroxyls. These include alkyl halides, such as methyl iodide, methyl bromide, ethyl chloride, propyl iodide; aralkyl halides such as benzyl chloride and methyl-benzyl chloride; hydroxyalkylchlorides such as hydroxyethyl chloride; carboxyalkylating agents such as sodium monochloracetate; and alkylene halides such as allyl chloride. Ordinarily, the etherification is carried out in strongly basic environments; sodium hydroxide, liquid ammonia and quaternary ammonium bases and salts being the usual basic substances present.

Esterification of the terminal hydroxyls may be accomplished with various inorganic groups such as nitrates, phosphates or sulfates. However, preferred esterifying agents are the organic acids anhydrides or acid chlorides, and especially fatty acid anhydrides and their chlorides, including for example formic, acetic, propionic, butyric, hexoic, 2-ethylhexoic, and higher fatty acids such as lauric, stearic, myristic, palmitic and capric acids. Usually, the esters are formed by treatment of the hydroxylated disulfide with the anhydride of the acid in the presence of a catalyst such as sulfuric or phosphoric acid. The saturated fatty acids form the most stable esters with the bis(hydroxy alkyl)disulfides.

At times it is preferable to allow only partial etherification, thus forming half-ethers or half-esters instead of the di-ethers or di-esters theoretically possible. For other purposes the end-group hydroxyls may not only be partially or completely esterified or etherified, but also may be so treated as to result in the formation of mixed ethers, mixed esters or ether-esters.

The disulfide lubricants comprise one or more compounds having the general configuration



wherein X is a substituent such as a hydrogen atom, hydrocarbon radical or acyl group, and each R is an organic radical, especially a hydrocarbon radical. It will be noted that disulfides having ether or ester end-groups may be formed from mercapto alkyl alcohols, etherification or esterification being effected subsequent to the formation of the disulfide, or they may be formed by oxidation of salts of mercapto-ethers or esters. Typical disulfide lubricants include one or more of the following: bis(3-hydroxypropyl)disulfide, bis(2-hydroxyethyl)disulfide, bis(3-methoxypropyl)disulfide, bis(2-ethoxyethyl)disulfide, bis(3-ethoxyloxypropyl)disulfide, bis(2-butoxyloxy)disulfide, 3-hydroxypropyl-2-hydroxyethyl disulfide and their homologs and analogs.

The lubricants of the present invention vary from thin liquids to viscous oils, and, dependent upon their configuration, some of the disulfides are gels or solids at room temperature. They have viscosities, viscosity indices, corrosion char-

acteristics, oxidation resistance, extreme pressure characteristics and lubricating properties which make them especially useful for lubricating purposes, either by themselves or in combination with other lubricants or lubricant additives.

The disulfide lubricants have pour points which make them useful over wide temperature ranges, some of them being particularly useful as low temperature lubricants, since they may have pour points as low as -65° F. or even lower. This property will depend to a certain extent on the molecular weight of the radicals attached to the disulfide group, and partly upon the structure of such radicals.

The disulfide lubricants have viscosities which vary over a considerable range, commonly being from about 10 to 500 centistokes at 100° F., and from 50 to 75 centistokes at 210° F. These viscosities correspond approximately to SAE 10-80 lubricating oils.

The resistance of the disulfide lubricants to oxidation and their response to oxidation inhibitors is outstanding. In this regard, one feature of the oxidation of the disulfide lubricants is that their products of oxidation are more or less volatile, and eventually tend to escape from the lubrication system, thus promoting engine cleanliness. This phenomenon is contrary to that experienced with mineral oils, which tend to form gums, sludge and lacquers upon oxidation, thereby causing corrosion, wear and consequent unsatisfactory engine operation. The disulfide lubricants respond particularly well to such oxidation inhibitors as 1,2-dihydroxybenzene, monocyclic paraphenylenediamines, monocyclic aminophenols, etc.

The outstanding properties of the disulfide lubricants is their superior performance as extreme pressure lubricants. This property is evident when the disulfides are used alone or when they are employed as extreme pressure additives for other lubricants such as mineral oils, polymers of alkylene oxides and glycols, polyamides, polymeric siloxanes, etc. The extreme pressure characteristic is especially outstanding when the blends of the disulfides and other lubricants contain from about 3 to 50% of the disulfides.

The disulfide lubricants may contain other substances to modify their properties, such as corrosion inhibitors (especially organic monobasic and polybasic acids which are capable of forming water-insoluble metallic salts), gelling agents for the formation of greases, etc. The lubricant compositions are useful as or in cutting oils as well as in engine lubricants.

Having described the preparation, properties and uses of the disulfide lubricants, illustrative examples are presented:

#### EXAMPLE I

##### *Preparation of bis(gamma-hydroxypropyl)disulfide*

Ninety-two parts gamma-mercaptopropyl alcohol were treated with 56 parts potassium hydroxide in aqueous solution. To the solution of the potassium salt so formed, 126 parts iodine were added dropwise, starting at room temperature. The product so formed was water-washed and unreacted material was removed by fractional distillation in order to recover bis(gamma-hydroxypropyl) disulfide.

The disulfide was used as an extreme pressure additive, as described in Example II.

7  
EXAMPLE II

*Use of disulfide as an extreme pressure agent*

The extreme pressure characteristics of the disulfide prepared as described in Example I were tested, using the 4-ball machine described by Boelage in "Engineering", July 14, 1933. The tests comprise determining the wear caused by use of a propylene oxide polymeric lubricant, both in the presence and absence of the disulfide. The results obtained are given below. The conditions used were one minute at 1500 R. P. M. under the indicated loads.

| Weight percent disulfide in lubricant | Scar Diameters (mm.) |      |      |      |
|---------------------------------------|----------------------|------|------|------|
|                                       | 0                    | 0.62 | 2.8  | 3.2  |
| Load (kg.):                           |                      |      |      |      |
| 40                                    | 0.35                 |      |      |      |
| 60                                    | 0.57                 | 0.48 |      | 0.46 |
| 80                                    | 1.63                 | 0.54 |      | 0.57 |
| 100                                   | 2.50                 | 0.66 |      | 0.73 |
| 140                                   | Weld                 | 1.85 | 0.89 | 1.17 |
| 200                                   |                      | 2.63 | 1.93 | 1.99 |
| 300                                   |                      | 2.50 |      | 2.53 |
| 400                                   |                      | 3.59 |      | 3.28 |
| 500                                   |                      | Weld | 3.88 | 3.90 |
| 600                                   |                      |      | Weld | 3.91 |
| 700                                   |                      |      |      | Weld |

We claim as our invention

1. A lubricating composition comprising a major amount of an oleaginous alkylene polymeric oxide material and a minor amount sufficient to impart extreme pressure properties of an organic disulfide having the general configuration:  $XO-R-S-S-R-OX$ , wherein each R is a saturated alkylene radical and each X is a substituent of the group consisting of hydrogen atoms, saturated alkyl radicals and saturated acyclic acyl groups having up to eighteen carbon atoms, said disulfide being prepared by dispersing a mercapto alkyl monohydric alcohol in an alkaline medium, oxidizing said alcohol with a peroxide, removing from the product the portion volatilizing below about 140° C. at 0.2 cm. mercury pressure to obtain the organic disulfide residue.

2. A lubricating composition comprising a major amount of an oleaginous alkylene polymeric oxide material and a minor amount sufficient to impart extreme pressure properties of an organic disulfide having the general configuration:  $XO-R-S-S-R-OX$ , wherein each R is a saturated alkylene radical and each X is a substituent of the group consisting of hydrogen atoms, saturated alkyl radicals and saturated acyclic acyl groups having up to eighteen carbon atoms, said disulfide being prepared by dispersing a mercapto alkyl monohydric alcohol in an alkaline medium, oxidizing said alcohol with a halogen, removing from the product the portion volatilizing below about 140° C. at 0.2 cm. mercury pressure to obtain the organic disulfide residue.

3. A lubricating composition consisting essentially of an oleaginous propylene oxide polymer and as an extreme pressure agent therefor from 0.62 to 3.2% by weight of bis(gamma-hydroxypropyl) disulfide, which disulfide has a boiling point of at least about 140° C. at 0.2 cm. mercury pressure.

4. A lubricating composition consisting essentially of an oleaginous alkylene polymeric oxide material and a minor amount sufficient to impart extreme pressure properties of bis(beta-hydroxyethyl) disulfide, which disulfide has a boiling point of at least about 140° C. at 0.2 cm. mercury pressure.

5. A lubricating composition consisting essentially of an oleaginous alkylene polymeric oxide material and a minor amount sufficient to impart extreme pressure properties of bis(gamma-hydroxypropyl) disulfide, which disulfide has a boiling point of at least about 140° C. at 0.2 cm. mercury pressure.

6. A lubricating composition consisting essentially of an alkylene polymeric oxide material and a minor amount sufficient to impart extreme pressure properties of an organic disulfide residue having the general configuration:



15 wherein  $A_1$  and  $A_2$  are saturated acyclic acyl groups having up to eighteen carbon atoms and  $R_1$  and  $R_2$  are saturated alkylene radicals, said disulfide being prepared by dispersing a mercapto alkyl monohydric alcohol in an alkaline medium, oxidizing said alcohol, and removing from the product the portion volatilizing below about 140° C. at 0.2 cm. mercury pressure to obtain the organic disulfide residue.

20 7. A lubricating composition consisting essentially of an oleaginous alkylene polymeric oxide material and a minor amount sufficient to impart extreme pressure properties of an organic disulfide residue having the general configuration:  $R_1-O-R_2-S-S-R_3-O-R_4$ , wherein  $R_1$  and  $R_4$  are saturated alkyl radicals having up to four carbon atoms and  $R_2$  and  $R_3$  are saturated alkylene radicals, said disulfide being prepared by dispersing a mercapto alkyl monohydric alcohol in an alkaline medium, oxidizing said alcohol, and  $35$  removing from the product the portion volatilizing below about 140° C. at 0.2 cm. mercury pressure to obtain the organic disulfide residue.

25 8. A lubricating composition consisting essentially of an oleaginous alkylene polymeric oxide material and a minor amount sufficient to impart extreme pressure properties of an organic disulfide residue having the general configuration:  $HO-R_1-S-S-R_2-OH$ , wherein  $R_1$  and  $R_2$  are saturated alkylene radicals, said disulfide being prepared by dispersing a mercapto alkyl monohydric alcohol in an alkaline medium, oxidizing said alcohol, and removing from the product the portion volatilizing below about 140° C. at 0.2 cm. mercury pressure to obtain the organic disulfide residue.

30 9. A lubricating composition consisting essentially of a major amount of an oleaginous alkylene polymeric oxide material and a minor amount sufficient to impart extreme pressure properties of an organic disulfide residue having the general configuration:  $XO-R-S-S-R-OX$ , wherein each R is a saturated alkylene radical and each X is a substituent of the group consisting of hydrogen atoms, saturated alkyl radicals and  $35$  saturated acyclic acyl groups having up to eighteen carbon atoms, said disulfide being prepared by dispersing a mercapto alkyl monohydric alcohol in an alkaline medium, oxidizing said alcohol, and removing from the product the portion volatilizing below about 140° C. at 0.2 cm. mercury pressure to obtain the organic disulfide residue.

35 10. A lubricating composition consisting essentially of a major amount of an oleaginous propylene oxide polymer and a minor amount sufficient to impart extreme pressure properties of an organic disulfide residue of the group consisting of bis(hydroxy alkyl) disulfides having the general configuration:  $HO-R-S-S-R-OH$ , wherein  $40$   $R$  is a saturated alkylene radical, said disulfide

being prepared by dispersing a mercapto alkyl monohydric alcohol in an alkaline medium and oxidizing said alcohol; saturated alkyl ethers thereof; and saturated acyclic esters thereof, the acyl groups of said esters having up to 18 carbon atoms, said residue having removed therefrom any portion volatilizing below 140° C. at 0.2 cm. mercury pressure.

WILLIAM E. VAUGHAN.  
DENHAM HARMAN.

10  
REFERENCES CITED

The following references are of record in the file of this patent:

## UNITED STATES PATENTS

| Number    | Name           | Date           |
|-----------|----------------|----------------|
| 2,001,715 | Fischer        | May 21, 1935   |
| 2,174,248 | Mikeska et al. | Sept. 26, 1939 |
| 2,246,712 | Barth          | June 24, 1941  |
| 2,293,868 | Toussaint      | Aug. 25, 1942  |
| 2,378,576 | Okita          | June 19, 1945  |
| 2,415,002 | Bruson         | Jan. 28, 1947  |